

## UNITED STATES PATENT OFFICE

2,121,292

MAGNESIUM ALLOYS CONTAINING CERIUM  
AND OTHER ELEMENTSJohn Leslie Haughton and William Eliezer  
Prytherch, Teddington, EnglandNo Drawing. Application April 20, 1937, Serial  
No. 138,064. In Great Britain May 5, 1936

## 1 Claim. (Cl. 75—168)

This invention relates to magnesium alloys rich in magnesium.

The present invention is based upon the observation that beneficial effects are secured by the incorporation in magnesium alloys rich in magnesium of a proportion of cerium and a proportion of one or more of the metals, nickel, manganese and cobalt and optionally also a proportion of calcium, and further that instead of using metallic cerium mixtures of rare earth metals containing cerium may be used, for instance a mixture of cerium and thorium or the mixture known as "Mischiometall" which is a mixture of rare earth metals containing about 60 to 70% of cerium.

The invention consists in ternary or higher magnesium alloys rich in magnesium containing one or more of the metals, nickel, manganese and cobalt and in addition cerium and optionally also calcium.

The invention further extends to ternary or higher magnesium alloys rich in magnesium containing nickel, manganese or cobalt in the presence or absence of calcium and in addition a proportion of cerium in association with other rare earth metals, for instance, thorium and in particular the rare earth metals present with cerium in the mixture known as "Mischiometall".

The invention consists more particularly in magnesium rich alloys containing up to about 12 per cent. of cerium and of one or more of the metals, nickel, manganese and cobalt up to the proportion of, say, 8 per cent.

Normally the minimum proportions of cerium present in alloys in accordance with the invention is in the neighbourhood of 2 per cent. while the minimum proportion of the metals, nickel and cobalt is normally not less than 1 per cent. and the minimum content of manganese not less than 0.1 per cent. Where calcium is present the minimum proportion thereof in the alloy is normally not less than 0.1 per cent. and the proportion thereof may vary from this limit to, say, 5 per cent.

The invention further extends to articles formed from such alloys and the heat treatment of such alloys and articles in the manner hereinafter defined.

The following particulars are given by way of example to illustrate the properties of particular alloys within the scope of the invention, it being

understood that the invention is not restricted to alloys of the particular compositions stated in the examples:—

## Example I

Nominal composition: Cerium 6%, nickel 6%, magnesium remainder.

|                                                      |       |
|------------------------------------------------------|-------|
| Ultimate stress, room temperature (tons per sq. in.) | 15.02 |
| Ultimate stress, 200° C. (tons per sq. in.)          | 13.6  |
| Ultimate stress, 300° C. (tons per sq. in.)          | 6.7   |

## Example II

Nominal composition: Cerium 3%, nickel 6%, manganese 1.25%, magnesium remainder.

|                                                      |      |
|------------------------------------------------------|------|
| Ultimate stress, room temperature (tons per sq. in.) | 17.7 |
| Ultimate stress, 200° C. (tons per sq. in.)          | 12.6 |
| Ultimate stress, 300° C. (tons per sq. in.)          | 6.1  |

## Example III

Nominal composition: Cerium 6%, manganese 1.25%, magnesium remainder.

|                                                      |      |
|------------------------------------------------------|------|
| Ultimate stress, room temperature (tons per sq. in.) | 18.2 |
| Ultimate stress, 200° C. (tons per sq. in.)          | 11.0 |
| Ultimate stress, 300° C. (tons per sq. in.)          | 5.9  |

## Example IV

Nominal composition (approximate only): Cerium 3%, manganese 1%, cobalt 2%, calcium 0.5%, magnesium remainder.

| Temperature      | Brinell hardness number |
|------------------|-------------------------|
| Room temperature | 55.0                    |
| 200° C.          | 41.3                    |
| 300° C.          | 29.0                    |

For the purposes of comparison there may be quoted the following properties of an alloy containing cerium 6%, calcium 1% and the remainder magnesium.

|                                                              |      |
|--------------------------------------------------------------|------|
| Ultimate tensile stress, room temperature (tons per sq. in.) | 16.4 |
| Ultimate tensile stress, 200° C. (tons per sq. in.)          | 11.5 |
| Ultimate tensile stress, 300° C. (tons per sq. in.)          | 6.1  |

The alloys may be prepared by adding the cerium, calcium, nickel, manganese or cobalt, 50

either as metals or as magnesium-rich alloys, to the molten magnesium or the cerium may be added in the form of the alloys previously mentioned.

5 Some improvement in properties results from a heat treatment of the alloys. The heat treatment may consist of (I) heating the alloys to about 500° C. or higher, and then (II) hardening by heating to a lower temperature, say, 130-220° C.

10 for one or more days. The heat treatment is, however, not essential in

producing alloys possessing desirable properties.

We claim:

Magnesium rich alloys containing between 2 and 12 per cent. of cerium, a proportion of 0.1 to 8 per cent. of at least one metal selected from the 5 group nickel and cobalt, a proportion of manganese of between 0.1 to 4 per cent., and a proportion of calcium up to 5 per cent., the balance being magnesium.

JOHN LESLIE HAUGHTON.  
WILLIAM ELIEZER PRYTHERCH.

10